



US008889329B1

(12) **United States Patent**  
Veregin et al.

(10) **Patent No.:** US 8,889,329 B1  
(45) **Date of Patent:** Nov. 18, 2014

(54) **ALUMINA NANOTUBES AS A TONER ADDITIVE TO REDUCE IMPACTION**

(71) Applicant: **Xerox Corporation**, Norwalk, CT (US)

(72) Inventors: **Richard P. N. Veregin**, Mississauga (CA); **Padam K. Angra**, Pittsford, NY (US)

(73) Assignee: **Xerox Corporation**, Norwalk, CT (US)

(\*) Notice: Subject to any disclaimer, the term of this patent is extended or adjusted under 35 U.S.C. 154(b) by 16 days.

(21) Appl. No.: 13/903,293

(22) Filed: May 28, 2013

(51) **Int. Cl.**

**G03G 9/097** (2006.01)  
**G03G 9/08** (2006.01)

(52) **U.S. Cl.**

CPC ..... **G03G 9/08** (2013.01)  
USPC ..... **430/108.3; 430/108.6**

(58) **Field of Classification Search**

USPC ..... 430/108.3, 108.6  
See application file for complete search history.

(56) **References Cited**

U.S. PATENT DOCUMENTS

|              |         |                   |
|--------------|---------|-------------------|
| 4,295,990 A  | 10/1981 | Verbeek et al.    |
| 4,457,998 A  | 7/1984  | Gruber et al.     |
| 4,935,326 A  | 6/1990  | Creatura et al.   |
| 4,937,166 A  | 6/1990  | Creatura et al.   |
| 5,290,654 A  | 3/1994  | Sacripante et al. |
| 5,302,486 A  | 4/1994  | Patel et al.      |
| 5,556,732 A  | 9/1996  | Chow              |
| 6,042,981 A  | 3/2000  | Barbetta et al.   |
| 6,063,827 A  | 5/2000  | Sacripante et al. |
| 6,355,391 B1 | 3/2002  | Van Dusen et al.  |
| 6,593,049 B1 | 7/2003  | Veregin et al.    |

|                   |         |                                |
|-------------------|---------|--------------------------------|
| 6,756,176 B2      | 6/2004  | Stegamat et al.                |
| 6,830,860 B2      | 12/2004 | Sacripante et al.              |
| 7,014,971 B2      | 3/2006  | Skorokhod et al.               |
| 7,485,400 B2      | 2/2009  | Veregin et al.                 |
| 7,524,602 B2      | 4/2009  | Vanbesien et al.               |
| 2010/0040969 A1 * | 2/2010  | Bejat et al. .... 430/111.1    |
| 2010/0124713 A1 * | 5/2010  | Farrugia et al. .... 430/108.1 |

OTHER PUBLICATIONS

Cheng et al, "Al<sub>2</sub>O<sub>3</sub>:Cr<sup>3+</sup> nanotubes synthesized via homogenization precipitation followed by heat treatment", Journal of Physical Chemistry B, 110, (2006), pp. 15749-15754.

Dahlan et al., "γ-Alumina Nanotubes Prepared by Hydrothermal Method as Support of Iron, Cobalt and Nickel for Fischer-Tropsch Catalysts" Chemistry and Materials Research, Online, vol. 2, No. 3, 2012, pp. 31-39.

Lihong Qu et al., "Hydrothermal synthesis of alumina nanotubes templated by anionic surfactant", Materials Letters, vol. 59, Issues 29-30, Dec. 2005, pp. 4034-4037.

Woo Lee et al., "A Continuous Process for Structurally Well-Defined Al<sub>2</sub>O<sub>3</sub> Nanotubes Based on Pulse Anodization of Aluminum," American Chemical Society—Nano letters, vol. 8, No. 8, (2008), pp. 2155-2160.

Angra et al., "Toner Additives", U.S. Appl. No. 13/745,535, filed Jan. 18, 2013.

Veregin et al., "Toner Additives", U.S. Appl. No. 13/705,524, filed Dec. 5, 2012.

\* cited by examiner

Primary Examiner — Peter Vajda

(74) Attorney, Agent, or Firm — MH2 Technology Law Group LLP

(57)

**ABSTRACT**

The disclosure relates generally to toner additives, and in particular, toner additives that provide reduced impaction within a toner particle and improved adhesion to the toner particle. The toner additives include alumina nanotubes, and may be used with other non-conventional additives such as silica nanotubes and titania nanotubes.

21 Claims, 1 Drawing Sheet





## ALUMINA NANOTUBES AS A TONER ADDITIVE TO REDUCE IMPACTION

### TECHNICAL FIELD

The disclosure relates generally to toner additives, and in particular, toner additives that provide reduced impaction within toner particles. The toner additives comprise alumina nanotubes in combination with or in place of or in combination with the commonly used toner additives, such as alumina.

### BACKGROUND

In electrostatography, for example xerography, electrophotographic imaging or electrostatographic imaging, an imaging process may include forming a visible toner image on a support surface such as a paper sheet, plastics, films, etc. The visible toner image is often produced by forming a latent electrostatic image on a charged photoreceptor, which can be transferred to an intermediate transfer belt, and then fixed onto the support surface using a heated fuser belt or a heated roll fuser to form a permanent image.

Toners for imaging devices such as electrostatographic printers may include at least a binder resin, a colorant, and one or more external surface additives that may be added in small amounts. Examples of external surface additives include, for example, silica, titanium dioxide, zinc stearate and the like. The properties of a toner are influenced by the materials and amounts of the materials of the toner. The charging characteristics of a toner also can depend on the carrier used in a developer composition, such as the carrier coating.

Alumina ( $Al_2O_3$ ) is an example of a toner additive. A typical alumina particle has a crystalline structure and is generally of a similar size in all dimensions, with a rough exterior having, for example, sharp edges. An alumina particle is more charge neutral than either silica and titania. Alumina used as a toner additive has a mean diameter of between about 10 nanometer (nm) and about 200 nm. In certain instances, alumina may be used as a toner additive to lower negative charge or increase positive charge. Like most oxides, alumina may serve several purposes as an additive. For example, alumina may improve charge control, flow aid, and transfer aid, which in turn improves transfer of the toner from the photoreceptor to the intermediate transfer belt or from the intermediate transfer belt to the support surface.

Due to its small size, alumina may embed or impact into the surface of the toner under low throughput or high toner age conditions, and may therefore lose its effectiveness and result in a decrease in the development of the toner and the transfer efficiency of the toner from the photoreceptor to the support substrate to be printed. To overcome this problem, larger sized "spacer" additives may be used shield small size additives such as silica, titania and alumina from impacting into the toner surface. While using larger sized additives may improve the effectiveness of the smaller additives, they increase production costs and attach poorly to the toner surface. Further, the larger sized additives can contaminate various materials and structures, such as the developer material, developer housing, charging devices, photoreceptor, transfer devices, and fuser components.

Thus, there is a need for new surface additives that can provide high charge and reduced additive impaction with improved adhesion of the additive to the toner surface.

### SUMMARY

The following presents a simplified summary in order to provide a basic understanding of some aspects of one or more

embodiments of the present teachings. This summary is not an extensive overview, nor is it intended to identify key or critical elements of the present teachings nor to delineate the scope of the disclosure. Rather, its primary purpose is merely to present one or more concepts in simplified form as a prelude to the detailed description presented later.

In an embodiment, a toner composition can include toner particles comprising a resin and a colorant, and one or more surface additives applied to a surface of the toner particles, the one or more surface additives comprising alumina nanotubes.

In another embodiment, a toner composition can include toner particles comprising a resin and a colorant, and one or more surface additives applied to a surface of the toner particles, the one or more surface additives comprising alumina nanotubes, wherein the toner composition has a high charge of from about -15 microcoulomb per gram to about -80 microcoulomb per gram and a low relative humidity sensitivity ratio of from about 1 to about 2.

In another embodiment, a developer can include a toner composition and a toner carrier, wherein the toner composition comprises toner particles comprising a resin and a colorant, and one or more surface additives applied to a surface of the toner particles, the one or more surface additives comprising alumina nanotubes.

### BRIEF DESCRIPTION OF THE DRAWINGS

The accompanying drawings, which are incorporated in and constitute a part of this specification, illustrate embodiments of the present teachings and together with the description, serve to explain the principles of the disclosure. In the figures:

FIG. 1 is a schematic depiction of alumina nanotubes 35 adhering to the surface of a toner particle.

It should be noted that some details of the FIG. have been simplified and are drawn to facilitate understanding of the present teachings rather than to maintain strict structural accuracy, detail, and scale.

### DETAILED DESCRIPTION

Reference will now be made in detail to exemplary embodiments of the present teachings, examples of which are 45 illustrated in the accompanying drawings. Wherever possible, the same reference numbers will be used throughout the drawings to refer to the same or like parts.

As used herein, unless otherwise specified, the word "printer" encompasses any apparatus that performs a print outputting function for any purpose, such as a digital copier, bookmaking machine, facsimile machine, a multi-function machine, electrostatographic device, etc.

The disclosure relates toner additives that provide desired higher and stable toner charge. The toner additives include 55 alumina nanosheets and/or alumina nanotubes (hereinafter collectively, unless otherwise specified, alumina nanotubes "AlNTs") in place of or in combination with the commonly used alumina ( $Al_2O_3$ ) toner additives and other additives as described below. AlNT additives have a unique shape that allows them to provide flow aid and transfer aid to the toner. AlNTs have a narrow cylindrical structure that allows them to act like small particles in one dimension and adhere strongly to the toner surface, thereby reducing contamination of various xerographic equipment components. The longer dimension 60 of these AlNTs further allow them to act like large particles offering lower or no impaction into the toner surface under low, throughput or high toner age conditions, thus 65

delivering more consistent developability and transfer efficiency without the need for larger size spacer additives.

A toner including titania nanotubes is described in copending U.S. patent application Ser. No. 13/705,524, filed Dec. 5, 2012, and a toner including silica nanotubes is described in copending U.S. patent application Ser. No. 13/745,535, filed Jan. 18, 2013, each of which is commonly assigned and incorporated herein by reference in its entirety. An embodiment of the present teachings may include the use of a toner having a plurality of alumina nanotubes as an additive to result in a toner having desirable charging and release characteristics during a printing process, and may further include a toner having a plurality of alumina nanotubes in combination with titania nanotubes, silica nanotubes, or both titania nanotubes and silica nanotubes.

Alumina nanotubes according to embodiments of the present teachings have a long, narrow cylindrical shape that allows them to function in a particular manner. The narrow width allows the alumina nanotubes to adhere strongly to a surface of the toner, which prevents their dislodging from the toner surface during printing. As discussed above, dislodged particles, such as dislodged spherical alumina particles, may contaminate various xerographic structures or materials, such as developer material, developer housing, charging devices, photoreceptor, transfer devices, and fuser components. On the other hand, the longer dimension of alumina nanotubes would the alumina nanotubes to function as large particles so that little or no impaction into the toner surface occurs during low printer throughput or aging of the toner. Decreasing impaction may result in a toner with improved developing and better transfer efficiency.

FIG. 1 is a schematic depiction (not to scale) representing adherence of a plurality of alumina nanotubes 10 to a toner particle 12 (one of which is depicted in FIG. 1). Adhesion efficiency of the plurality of alumina nanotubes 10 to a plurality of toner particles 12 depends, for example, on the size and aspect ratio of the alumina nanotubes. Due to the morphology of the alumina nanotubes, the alumina nanotubes have a cylindrical shape that provides a high surface curvature in one dimension. Each alumina nanotube thus acts like a small particle because of its narrow width but, at the same time, the high aspect ratio (length/diameter), particularly the long length compared to the narrow width, increases a contact area between the surface of the alumina nanotube and the surface of the toner particles. This increased surface area may reduce impaction as it increases the adhesion of the additive to the toner surface, making it less likely to cause contamination of other subsystems.

In an embodiment, a mean length of a plurality of alumina nanotubes in accordance with the present teachings may be between about 50 nm and about 2,000 nm, or between about 100 nm and about 1000 nm, or between about 150 nm and about 500 nm. A mean width (diameter) of the plurality of alumina nanotubes in accordance with the present teachings may be between about 5 nm and about 100 nm, or between about 5 nm and about 50 nm, or between about 6 nm and about 20 nm.

A pull off force for an additive is proportional to its mass ( $F=ma$ ), while the adhesion force is proportional to the area in contact and the nature of the chemical interaction. In the absence of specific chemical bonds, the latter will simply be the van der Waal's forces which do not vary much with material composition. Thus, how well the additive sticks to the surface of the toner will depend mostly on the ratio of the surface area in contact to the mass, for alumina additives the surface area to volume, since density is the same for all. Thus, for example, a nanotube of 12 nm diameter and 500 nm length

as described below has the same surface area/mass ratio as a 17 nm spherical alumina particle. Thus the alumina nanotube adheres to the surface of a toner particle similar to a small titania. Also, since the alumina nanotube has a small radius in one dimension, in terms of properties like toner flow a nanotube acts like a small particle, and thus provides improved flow than a large particle, as cohesion is proportional to the particle radius. However, in terms of additive impaction, the area of an alumina nanotube in contact with a toner particle is equivalent to that of a larger particle, and it is more difficult for alumina nanotubes to impact within the toner particle. Thus for impaction, the alumina nanotubes above are the equivalent of a 55 nm spherical alumina. As the alumina nanotube becomes longer, these desirable effects increase. The overall effect is that for charge, flow, and adhesion to the toner, alumina nanotubes have the desirable characteristics of small particles while, for impaction, the alumina nanotubes have the desirable characteristics of large particles.

Thus alumina nanotubes as toner additives and, in particular, as surface toner additives are advantageous over commonly used alumina particles. Due to their unique shape and large aspect ratio they are expected to attach strongly to the toner surface and eliminate the contamination of the developer material, developer housing, charging devices, photoreceptor, transfer devices, and fuser components. They are also expected to impact less into the toner surface and deliver consistent developability and transfer efficiency under low throughput conditions. Due to the different chemistry of alumina compared to silica and titania, the alumina will provide the opportunity to have less of an effect on the overall charging of the toner, or lowering the charge compared to silica and titania in negative toner developers, or providing positive charge for positive toner developers.

Alumina nanotubes can be prepared in different morphologies using any suitable processes. For example, the preparation of alumina nanotubes are discussed in the following references, each of which is incorporated by reference in its entirety: 1) Cheng, B., Qu, S., Zhou, H., & Wang, Z. (2006), “ $\text{Al}_2\text{O}_3:\text{Cr}^{3+}$  nanotubes synthesized via homogenization precipitation followed by heat treatment”, *Journal of Physical Chemistry B*, 110, 15749-15754; 2) Dahlani, I Nyoman Marsih, IGBN Makerti Hartha, Piyasan Praserthdam, Joongjai Panpranon, Ismunandary, “Alumina Nanotubes Prepared by Hydrothermal Method as Support of Iron, Cobalt and Nickel for Fischer-Tropsch Catalysts” *Chemistry and Materials Research*, Online, Vol 2, No. 3, 31-39, 2012; 3) Lihong Qu, Changqing He, Yue Yang, Yanli He, Zhongmin Liu, “Hydrothermal synthesis of alumina nanotubes templated by anionic surfactant”, *Materials Letters*, Volume 59, Issues 29-30, December 2005, Pages 4034-4037; 4) Woo Lee, Roland Scholz and Ulrich Go, “A Continuous Process for Structurally Well-Defined  $\text{Al}_2\text{O}_3$  Nanotubes Based on Pulse Anodization of Aluminum,” *Nano letters*, Vol. 8, No. 8, 2155-2160 (2008).

Reference 3) above prepares alumina nanotubes having an outer diameter of 6 nm to 8 nm in outer diameter and up to 200 nm in length. To form alumina nanotubes, 2.8 g of sodium dodecyl sulfonate was dissolved into 70 g of distilled water at 50° C. to prepare solution A. 22.9 g of  $\text{Al}(\text{NO}_3)_3 \cdot 9\text{H}_2\text{O}$  was dissolved in 40 g of distilled water at room temperature to achieve solution B. Solution B was slowly added into solution A under stirring, and the mixture was continuously stirred for several minutes at 50° C. Thereafter, 12.0 g of aqueous ammonia was dripped into the mixture until pH value of 5.0-5.5. After being stirred for additional several minutes, the resulting suspension was transferred into a Teflon-lined autoclave (100 ml), and heated at 120° C. for 90 h. After the completion of hydrothermal treatment, the autoclave was

cooled down to room temperature naturally, and the solid product was recovered by centrifuge, washed several times with a solution consisting of distilled water and 95% ethanol, and finally dried at 50° C. overnight. The template in the solids was removed by calcinations and extraction, respectively. During calcinations, the sample was heated in air from room temperature to a certain temperature in the range of 500-800° C. with a temperature ramp of 1° C. min<sup>-1</sup>, and kept at that temperature for 5 h. 0.2 M ethanol solution of ammonium acetate was used to perform the solvent extraction at room temperature for 4 days while stirring.

Reference 4) above prepares alumina nanotubes having an outer diameter of about 95 nm in diameter while the length is controllable by tuning the pulse in the anodization.

In the present embodiments, the toner with alumina nanotubes has excellent toner flow. Toner flow can be measured as described in U.S. Pat. No. 7,485,400, which is hereby incorporated by reference in its entirety, providing a cohesion of from about 10% to about 40%, or from about 20% to about 70%, or from about 10% to 73%.

In the present embodiments, the toner with alumina nanotubes may provide high adhesion of the nanotubes to the toner particle, so that the alumina nanotubes remain on the toner particle during the print process. The adhesion of the alumina nanotubes to the toner particle can be measured as described in U.S. Pat. No. 7,485,400, which is hereby incorporated by reference in its entirety, providing an Additive Adhesion Force Distribution (AAFD) percent value of greater than about 40% at energy of sonification of 12 kilojoules of energy, at from about 10 to 12 minutes of sonification. In embodiments, the AAFD can have a value of greater than about 40% at 6 kilojoules of energy, at from about 5 to 6 minutes of sonification, and in further embodiments, the AAFD can have a value of 40% at 3 kilojoules of energy, at from about 2.5 to 3 minutes of sonification.

In embodiments, the toner made from the present embodiments maintains a high charge of from about -15 to about -80 microcoulombs/gram or from about -20 to about -70 microcoulombs/gram or from about -20 to about -60 microcoulombs/gram.

In the present embodiments, there is provided a toner composition comprising alumina nanotubes. The toners may be prepared by chemical methods (emulsion/aggregation) and physical methods (grinding), both of which may be equally employed. Thus, the toner may be any conventional toner. In specific embodiments, the toner may also be an emulsion aggregate toner. In embodiments, these alumina nanotubes are included on the toner surface as toner surface additives. The alumina nanotubes are included in place of, or in combination with, other conventional toner surface additives, such as for example, particulate silica, titania, or alumina. Further, it is contemplated that the alumina nanotubes may be used in combination with silica nanotubes, titania nanotubes, or both silica nanotubes and titania nanotubes.

As described above, the alumina nanotubes have structures that may be cylindrical—spherical in one dimension and more linear in other dimensions. In embodiments, the alumina nanotubes have an average particle diameter of from about from about 5 nm to about 100 nm, or from about 5 to about 50 nm, or from about 6 to about 20 nm. In embodiments, the alumina nanotubes have an average particle length of from about from about 50 nm to about 2 microns, or from about 100 nm to about 1 micron, or from about 150 nm to about 500 nm.

In further embodiments, the alumina nanotubes are present in an amount of from about 0.1 wt % to about 5 weight percent (wt %), or from about 0.5 wt % to about 3 wt %, or of from

about 1 wt % to about 4 wt % by weight of the total weight of the toner particle including additives. In other embodiments, the alumina nanotubes are used in combination with the conventional particulate toner surface additives. In such embodiments, the alumina nanotubes are present in an amount of from about 0.1 wt % to about 5 wt %, or of from about 0.5 wt % to about 3 wt %, or of from about 1 wt % to about 4 wt % by weight of the total weight of the toner particle while the conventional toner surface additives are present in an amount of from about 0.1 wt % to about 5 wt %, or of from about 0.5 wt % to about 3 wt %, or of from about 1 wt % to about 4 wt % by weight of the total weight of the toner particle including additives. The conventional toner surface additives may be selected from the group consisting of SiO<sub>2</sub>, or metal oxides such as TiO<sub>2</sub> and AlO<sub>2</sub>, and mixtures thereof. The particulate titania may be of anatase or rutile structure. The conventional toner surface additives may be surface treated. In embodiments, the toner comprises at least one of a silica and a titania additive, where the silica comprises between 0.1 wt % and 4 wt % of the toner composition, or from 0.5 wt % to 3 wt % of the toner composition; the titania comprises between 0.1 wt % and 3 wt % of the toner composition, or about 0.5% to about 2 wt % of the toner composition; and the alumina nanotubes comprise between 0.1 wt % and 5 wt % of the toner composition, or about 0.5 wt % to about 4 wt % of the toner composition, or about 1 wt % to about 3 wt % of the toner composition; and where the total additive loading comprises about 0.3 wt % of the toner composition to about 8 wt % of the toner composition, or about 1 wt % of the toner composition to about 6 wt % of the toner composition, or about 2 wt % of the toner composition to about 5 wt % of the toner composition.

In addition, the alumina nanotubes may be used in combination with non-conventional toner surface additives such as silica nanotubes and/or titania nanotubes. If used with only one of silica nanotubes and titania nanotubes, the alumina nanotubes may be present in an amount of from about 0.1 wt % to about 5 wt %, or from about 0.5 wt % to about 4 wt %, or from about 1 wt % to about 3 wt %. The total additive loading may be from about 0.2 wt % to about 8 wt %.

If alumina nanotubes are used in combination with both silica nanotubes and titania nanotubes, each of the three material may be present in an amount of from about 0.1 wt % to about 3 wt %, or from about 0.2 wt % to about 2.5 wt %, or from about 0.4 wt % to about 2 wt %. The total additive loading may be from about 0.3 wt % to about 8 wt %.

Further, alumina nanotubes may be present in a different amount compared to either silica nanotubes and/or titania nanotubes. Because alumina nanotubes are generally charge neutral, silica nanotubes and/or titania nanotubes may be added in greater or lesser amounts to tailor the overall charge of the toner particle. Thus, in embodiments where the alumina nanotubes provides a low charge to the system, the alumina nanotubes may be added to supply a spacer function, whose benefits include preventing impaction of the other additives into the toner surface and improving the resistance of the toner composition to blocking of the toner particles, where the toner particles tend to stick together after exposure to high temperature. In such embodiments, the alumina nanotubes are present in amounts from about 0.5 wt % to 5 wt %, or about 1 wt % to about 4 wt %, or about 1.5% to about 3 wt % of the toner composition. Silica, including silica nanotubes, in general are expected to charge strongly negative, thus in embodiments they are added to the toner composition to increase the overall negative charge level. Thus, in embodiments where the silica is added to increase negative charge, the silica may be present in amounts from about 0.1 wt % to

about 4 wt %, or from about 0.5 wt % to about 3 wt %, or from about 1 wt % to about 2.5 wt %. However, silicas tend to be sensitive to relative humidity (RH) such that charge tends to decrease with increasing relative humidity. Thus, in the case where the silica nanotubes result in relative humidity sensitivity that is higher than desired then titania nanotubes may be added to the formulation. In general titania tends to provide lower negative charge than silica, but is less sensitive to relative humidity. Thus titania nanotubes may be added to the formulation to improve the relative humidity sensitivity of the toner composition, where the titania nanotubes may be added in the range of about 0.1 wt % to about 4 wt %, or from about 0.5 wt % to about 3 wt %, or from about 1 wt % to about 2.5 wt % of the toner composition. Thus, in embodiments, the alumina nanotubes provide impaction and blocking resistance without affecting the charge level of the toner composition, while the silica provides high charge and the titania provides improved RH level. Thus the impaction, charge and RH sensitivity of the toner may be varied independently giving flexibility to the toner design without compromising one performance attribute for another performance attribute. In these embodiments the silica and titania nanotubes may be replaced by conventional silica and titania toner additives, providing similar benefits for independently varying the additive impaction with the alumina nanotubes, the negative charge level with the silica and the relative humidity sensitivity with the titania. However, where the alumina, silica and titania are all nanotubes then the all the additives are resistant to additive impaction and toner blocking, and as well will adhere to the surface of the toner better than the conventional silica, titania and alumina additives, thus overall impaction will be improved and the presence of loose additives that are lost from the toner will be substantially reduced leading to less contamination of other subsystems in the electrophotographic printer.

In embodiments, the alumina nanotubes may be positively charging. In embodiments the alumina nanotubes may be added to create a positive charging toner composition, in effective amounts from about 0.1 wt % to 5 wt %, or about 0.5 wt % to about 4 wt %, or about 1 wt % to about 3 wt %. In embodiments, other positively charging charge enhancing additives may be added with the alumina nanotubes, including quaternary ammonium salts, including distearyl dimethyl ammonium methyl sulfate (DDAMS), and cetyl pyridinium chloride (CPC), combinations thereof, and the like, and other effective known charge agents or additives.

The alumina nanotubes may also be surface treated. In embodiments, the alumina nanotube are surface treated with compounds including dodecyltrimethoxysilane (DTMS) or hexamethyldisilazane (HMDS). Examples of these additives are alumina nanotubes coated with a mixture of HMDS and aminopropyltriethoxysilane, alumina nanotubes coated with PDMS (polydimethylsiloxane), alumina nanotubes coated with octamethylcyclotetrasiloxane, alumina nanotubes coated with dimethyldichlorosilane, DTMS alumina nanotubes comprising a alumina nanotubes core coated with DTMS, and alumina nanotubes coated with an amino functionalized organopolysiloxane.

#### Emulsion Aggregation Toner

In embodiments, a developer is disclosed including a resin coated carrier and a toner, where the toner may be an emulsion aggregation toner, containing, but not limited to, a latex resin, a wax and a polymer shell.

In embodiments, the latex resin may be composed of a first and a second monomer composition. Any suitable monomer or mixture of monomers may be selected to prepare the first monomer composition and the second monomer composi-

tion. The selection of monomer or mixture of monomers for the first monomer composition is independent of that for the second monomer composition and vice versa. Exemplary monomers for the first and/or the second monomer compositions include, but are not limited to, polyesters, styrene, alkyl acrylate, such as, methyl acrylate, ethyl acrylate, butyl acrylate, isobutyl acrylate, dodecyl acrylate, n-octyl acrylate, 2-chloroethyl acrylate;  $\beta$ -carboxy ethyl acrylate ( $\beta$ -CEA), phenyl acrylate, methyl alphachloroacrylate, methyl methacrylate, ethyl methacrylate and butyl methacrylate; butadiene; isoprene; methacrylonitrile; acrylonitrile; vinyl ethers, such as, vinyl methyl ether, vinyl isobutyl ether, vinyl ethyl ether and the like; vinyl esters, such as, vinyl acetate, vinyl propionate, vinyl benzoate and vinyl butyrate; vinyl ketones, such as, vinyl methyl ketone, vinyl hexyl ketone and methyl isopropenyl ketone; vinylidene halides, such as, vinylidene chloride and vinylidene chlorofluoride; N-vinyl indole; N-vinyl pyrrolidone; methacrylate; acrylic acid; methacrylic acid; acrylamide; methacrylamide; vinylpyridine; vinylpyrrolidone; vinyl-N-methylpyridinium chloride; vinyl naphthalene; p-chlorostyrene; vinyl chloride; vinyl bromide; vinyl fluoride; ethylene; propylene; butylenes; isobutylene; and the like, and mixtures thereof. In case a mixture of monomers is used, typically the latex polymer will be a copolymer.

In some embodiments, the first monomer composition and the second monomer composition may independently of each other comprise two or three or more different monomers. The latex polymer therefore can comprise a copolymer. Illustrative examples of such a latex copolymer includes poly(styrene-n-butyl acrylate- $\beta$ -CEA), poly(styrene-alkyl acrylate), poly(styrene-1,3-diene), poly(styrene-alkyl methacrylate), poly(alkyl methacrylate-alkyl acrylate), poly(alkyl methacrylate-aryl acrylate), poly(aryl methacrylate-alkyl acrylate), poly(alkyl methacrylate), poly(styrene-alkyl acrylate-acrylonitrile), poly(styrene-1,3-diene-acrylonitrile), poly(alkyl acrylate-acrylonitrile), poly(styrene-butadiene), poly(methylstyrene-butadiene), poly(methyl methacrylate-butadiene), poly(ethyl methacrylate-butadiene), poly(propyl methacrylate-butadiene), poly(butyl methacrylate-butadiene), poly(methyl acrylate-butadiene), poly(ethyl acrylate-butadiene), poly(propyl acrylate-butadiene), poly(butyl acrylate-butadiene), poly(styrene-isoprene), poly(methylstyrene-isoprene), poly(methyl methacrylate-isoprene), poly(ethyl methacrylate-isoprene), poly(propyl methacrylate-isoprene), poly(butyl methacrylate-isoprene), poly(methyl acrylate-isoprene), poly(ethyl acrylate-isoprene), poly(propyl acrylate-isoprene), poly(butyl acrylate-isoprene); poly(styrene-propyl acrylate), poly(styrene-butyl acrylate), poly(styrene-butadiene-acrylonitrile), poly(styrene-butyl acrylate-acrylonitrile), and the like.

In embodiments, the first monomer composition and the second monomer composition may be substantially water insoluble, such as, hydrophobic, and may be dispersed in an aqueous phase with adequate stirring when added to a reaction vessel.

The weight ratio between the first monomer composition and the second monomer composition may be in the range of from about 0.1:99.9 to about 50:50, including from about 0.5:99.5 to about 25:75, from about 1:99 to about 10:90.

In embodiments, the first monomer composition and the second monomer composition can be the same. Examples of the first/second monomer composition may be a mixture comprising styrene and alkyl acrylate, such as, a mixture comprising styrene, n-butyl acrylate and  $\beta$ -CEA. Based on total weight of the monomers, styrene may be present in an amount from about 1% to about 99%, from about 50% to about 95%, from about 70% to about 90%, although may be

present in greater or lesser amounts; alkyl acrylate, such as, n-butyl acrylate, may be present in an amount from about 1% to about 99%, from about 5% to about 50%, from about 10% to about 30%, although may be present in greater or lesser amounts.

In embodiments, the resins may be a polyester resin, such as, an amorphous resin, a crystalline resin, and/or a combination thereof, including the resins described in U.S. Pat. No. 6,593,049 and U.S. Pat. No. 6,756,176, the disclosure of each which is hereby incorporated by reference in its entirety. Suitable resins may also include a mixture of an amorphous polyester resin and a crystalline polyester resin as described in U.S. Pat. No. 6,830,860, the disclosure of which is hereby incorporated by reference in its entirety.

In embodiments, the resin may be a polyester resin formed by reacting a diol with a diacid in the presence of an optional catalyst. For forming a crystalline polyester, suitable organic diols include aliphatic diols with from about 2 to about 36 carbon atoms, such as 1,2-ethanediol, 1,3-propanediol, 1,4-butanediol, 1,5-pentanediol, 1,6-hexanediol, 1,7-heptanediol, 1,8-octanediol, 1,9-nonanediol, 1,10-decanediol, 1,12-dodecanediol and the like; alkali sulfo-aliphatic diols such as sodio 2-sulfo-1,2-ethanediol, lithio 2-sulfo-1,2-ethanediol, potassium 2-sulfo-1,2-ethanediol, sodio 2-sulfo-1,3-propanediol, lithio 2-sulfo-1,3-propanediol, potassium 2-sulfo-1,3-propanediol, mixture thereof, and the like. The aliphatic diol may be, for example, selected in an amount of from about 40 to about 60 mole percent, in embodiments from about 42 to about 55 mole percent, in embodiments from about 45 to about 53 mole percent (although amounts outside of these ranges can be used), and the alkali sulfo-aliphatic diol can be selected in an amount of from about 0 to about 10 mole percent, in embodiments from about 1 to about 4 mole percent of the resin.

Examples of organic diacids or diesters including vinyl diacids or vinyl diesters selected for the preparation of the crystalline resins include oxalic acid, succinic acid, glutaric acid, adipic acid, suberic acid, azelaic acid, sebacic acid, fumaric acid, dimethyl fumarate, dimethyl itaconate, cis, 1,4-diacetoxy-2-butene, diethyl fumarate, diethyl maleate, phthalic acid, isophthalic acid, terephthalic acid, naphthalene-2,6-dicarboxylic acid, naphthalene-2,7-dicarboxylic acid, cyclohexane dicarboxylic acid, malonic acid and mesaconic acid, a diester or anhydride thereof; and an alkali sulfo-organic diacid such as the sodio, lithio or potassium salt of dimethyl-5-sulfo-isophthalate, dialkyl-5-sulfo-isophthalate-4-sulfo-1,8-naphthalic anhydride, 4-sulfo-phthalic acid, dimethyl-4-sulfo-phthalate, dialkyl-4-sulfo-phthalate, 4-sulfo-phenyl-3,5-dicarbomethoxybenzene, 6-sulfo-2-naphthyl-3,5-dicarbomethoxybenzene, sulfo-terephthalic acid, dimethyl-sulfo-terephthalate, 5-sulfo-isophthalic acid, dialkyl-sulfo-terephthalate, sulfoethanediol, 2-sulfo-panediol, 2-sulfobutanediol, 3-sulfopentanediol, 2-sulfohexanediol, 3-sulfo-2-methylpentanediol, 2-sulfo-3,3-dimethylpentanediol, sulfo-p-hydroxybenzoic acid, N,N-bis(2-hydroxyethyl)-2-amino ethane sulfonate, or mixtures thereof. The organic diacid may be selected in an amount of, for example, in embodiments from about 40 to about 60 mole percent, in embodiments from about 42 to about 52 mole percent, in embodiments from about 45 to about 50 mole percent, and the alkali sulfo-aliphatic diacid can be selected in an amount of from about 1 to about 10 mole percent of the resin.

Examples of crystalline resins include polyesters, polyamides, polyimides, polyolefins, polyethylene, polybutylene, polyisobutylene, ethylene-propylene copolymers, ethylene-vinyl acetate copolymers, polypropylene, mixtures thereof,

and the like. Specific crystalline resins may be polyester based, such as poly(ethylene-adipate), poly(propylene-adipate), poly(butylene-adipate), poly(pentylene-adipate), poly(hexylene-adipate), poly(octylene-adipate), poly(ethylene-succinate), poly(propylene-succinate), poly(butylene-succinate), poly(pentylene-succinate), poly(hexylene-succinate), poly(octylene-succinate), poly(ethylene-sebacate), poly(propylene-sebacate), poly(butylene-sebacate), poly(pentylene-sebacate), poly(hexylene-sebacate), poly(octylene-sebacate), poly(decylene-sebacate), poly(decylene-decanoate), poly(ethylene dodecanoate), poly(nonylene-sebacate), poly(nonylene-decanoate), copoly(ethylene-fumarate)-copolymers(ethylene-sebacate), copoly(ethylene-fumarate)-copolymers(ethylene-decanoate), copoly(ethylene-fumarate)-copolymers(ethylene-dodecanoate), alkali copoly(5-sulfoisophthaloyl)-copolymers(ethylene-adipate), alkali copoly(5-sulfoisophthaloyl)-copolymers(propylene-adipate), alkali copoly(5-sulfoisophthaloyl)-copolymers(butylene-adipate), alkali copoly(5-sulfo-isophthaloyl)-copolymers(pentylene-adipate), alkali copoly(5-sulfo-isophthaloyl)-copolymers(hexylene-adipate), alkali copoly(5-sulfo-isophthaloyl)-copolymers(octylene-adipate), alkali copoly(5-sulfo-isophthaloyl)-copolymers(ethylene-succinate), alkali copoly(5-sulfoisophthaloyl)-copolymers(propylene-succinate), alkali copoly(5-sulfoisophthaloyl)-copolymers(butylene-succinate), alkali copoly(5-sulfoisophthaloyl)-copolymers(pentylene-succinate), alkali copoly(5-sulfoisophthaloyl)-copolymers(hexylene-succinate), alkali copoly(5-sulfoisophthaloyl)-copolymers(octylene-succinate), alkali copoly(5-sulfoisophthaloyl)-copolymers(ethylene-sebacate), alkali copoly(5-sulfo-isophthaloyl)-copolymers(ethylene-sebacate), alkali copoly(5-sulfo-isophthaloyl)-copolymers(hexylene-sebacate), alkali copoly(5-sulfo-isophthaloyl)-copolymers(octylene-sebacate), alkali copoly(5-sulfo-isophthaloyl)-copolymers(ethylene-adipate), alkali copoly(5-sulfo-isophthaloyl)-copolymers(butylene-adipate), alkali copoly(5-sulfo-isophthaloyl)-copolymers(pentylene-adipate), alkali copoly(5-sulfo-isophthaloyl)-copolymers(hexylene-adipate), poly(octylene-adipate), wherein alkali is a metal like sodium, lithium or potassium. Examples of polyamides include poly(ethylene-adipamide), poly(propylene-adipamide), poly(butylene-adipamide), poly(pentylene-adipamide), poly(hexylene-adipamide), poly(octylene-adipamide), poly(ethylene-succinimide), and poly(propylene-sebacamide). Examples of polyimides include poly(ethylene-adipimide), poly(propylene-adipimide), poly(butylene-adipimide), poly(pentylene-adipimide), poly(hexylene-adipimide), poly(octylene-adipimide), poly(ethylene-succinimide), poly(propylene-succinimide), and poly(butylene-succinimide).

The crystalline resin may be present, for example, in an amount of from about 5 to about 50 percent by weight of the toner components, in embodiments from about 10 to about 35 percent by weight of the toner components. The crystalline resin can possess various melting points of, for example, from about 30° C. to about 120° C., in embodiments from about 50° C. to about 90° C. The crystalline resin may have a number average molecular weight ( $M_n$ ), as measured by gel perme-

ation chromatography (GPC) of, for example, from about 1,000 to about 50,000, in embodiments from about 2,000 to about 25,000, and a weight average molecular weight ( $M_w$ ) of, for example, from about 2,000 to about 100,000, in embodiments from about 3,000 to about 80,000, as determined by Gel Permeation Chromatography using polystyrene standards. The molecular weight distribution ( $M_w/M_n$ ) of the crystalline resin may be, for example, from about 2 to about 6, in embodiments from about 3 to about 4.

Examples of diacids or diesters including vinyl diacids or vinyl diesters utilized for the preparation of amorphous polyesters include dicarboxylic acids or diesters such as terephthalic acid, phthalic acid, isophthalic acid, fumaric acid, dimethyl fumarate, dimethyl itaconate, cis, 1,4-diacetoxy-2-butene, diethyl fumarate, diethyl maleate, maleic acid, succinic acid, itaconic acid, succinic acid, succinic anhydride, dodecylsuccinic acid, dodecylsuccinic anhydride, glutaric acid, glutaric anhydride, adipic acid, pimelic acid, suberic acid, azelaic acid, dodecane diacid, dimethyl terephthalate, diethyl terephthalate, dimethylisophthalate, diethylisophthalate, dimethylphthalate, phthalic anhydride, diethylphthalate, dimethylsuccinate, dimethylfumarate, dimethylmaleate, dimethylglutarate, dimethyladipate, dimethyl dodecylsuccinate, and combinations thereof. The organic diacid or diester may be present, for example, in an amount from about 40 to about 60 mole percent of the resin, in embodiments from about 42 to about 52 mole percent of the resin, in embodiments from about 45 to about 50 mole percent of the resin. Examples of the alkylene oxide adducts of bisphenol include polyoxypropylene (2.2)-2,2-bis(4-hydroxyphenyl)propane, polyoxypropylene (3.3)-2,2-bis(4-hydroxyphenyl)propane, polyoxyethylene (2.0)-2,2-bis(4-hydroxyphenyl)propane, polyoxyethylene (2.2)-2,2-bis(4-hydroxyphenyl)propane, polyoxypropylene (2.0)-polyoxyethylene (2.0)-2,2-bis(4-hydroxyphenyl)propane, and polyoxypropylene (6)-2,2-bis(4-hydroxyphenyl)propane. These compounds may be used singly or as a combination of two or more thereof.

Examples of additional diols which may be utilized in generating the amorphous polyester include 1,2-propanediol, 1,3-propanediol, 1,2-butanediol, 1,3-butanediol, 1,4-butanediol, pentanediol, hexanediol, 2,2-dimethylpropanediol, 2,2,3-trimethylhexanediol, heptanediol, dodecanediol, 1,4-cyclohexanedimethanol, 1,3-cyclohexanedimethanol, xylenedimethanol, cyclohexanediol, diethylene glycol, dipropylene glycol, dibutylene, and combinations thereof. The amount of organic diol selected can vary, and may be present, for example, in an amount from about 40 to about 60 mole percent of the resin, in embodiments from about 42 to about 55 mole percent of the resin, in embodiments from about 45 to about 53 mole percent of the resin.

Polycondensation catalysts which may be utilized in forming either the crystalline or amorphous polyesters include tetraalkyl titanates, dialkyltin oxides such as dibutyltin oxide, tetraalkyltins such as dibutyltin dilaurate, and dialkyltin oxide hydroxides such as butyltin oxide hydroxide, aluminum alkoxides, alkyl zinc, dialkyl zinc, zinc oxide, stannous oxide, or combinations thereof. Such catalysts may be utilized in amounts of, for example, from about 0.01 mole percent to about 5 mole percent based on the starting diacid or diester used to generate the polyester resin.

In embodiments, suitable amorphous resins include polyesters, polyamides, polyimides, polyolefins, polyethylene, polybutylene, polyisobutylene, ethylene-propylene copolymers, ethylene-vinyl acetate copolymers, polypropylene, combinations thereof, and the like. Examples of amorphous resins which may be utilized include alkali sulfonated-poly-

ester resins, branched alkali sulfonated-polyester resins, alkali sulfonated-polyimide resins, and branched alkali sulfonated-polyimide resins. Alkali sulfonated polyester resins may be useful in embodiments, such as the metal or alkali salts of copoly(ethylene-terephthalate)-copoly(ethylene-5-sulfo-isophthalate), copoly(propylene-terephthalate)-copoly(propylene-5-sulfo-isophthalate), copoly(diethylene-terephthalate)-copoly(diethylene-5-sulfo-isophthalate), copoly(propylene-diethylene-terephthalate)-copoly(propylene-diethylene-5-sulfoisophthalate), copoly(propylene-butylene-terephthalate)-copoly(propylene-butylene-5-sulfo-isophthalate), copoly(propoxylated bisphenol-A-fumarate)-copoly(propoxylated bisphenol A-5-sulfo-isophthalate), copoly(ethoxylated bisphenol-A-fumarate)-copoly(ethoxylated bisphenol A-5-sulfo-isophthalate), and copoly(ethoxylated bisphenol-A-maleate)-copoly(ethoxylated bisphenol A-5-sulfo-isophthalate), wherein the alkali metal is, for example, a sodium, lithium or potassium ion.

In embodiments, as noted above, an unsaturated amorphous polyester resin may be utilized as a latex resin. Examples of such resins include those disclosed in U.S. Pat. No. 6,063,827, the disclosure of which is hereby incorporated by reference in its entirety. Exemplary unsaturated amorphous polyester resins include, but are not limited to, poly(propoxylated bisphenol co-fumarate), poly(ethoxylated bisphenol co-fumarate), poly(butyloxylated bisphenol co-fumarate), poly(co-propoxylated bisphenol co-ethoxylated bisphenol co-fumarate), poly(1,2-propylene fumarate), poly(propoxylated bisphenol co-maleate), poly(ethoxylated bisphenol co-maleate), poly(butyloxylated bisphenol co-maleate), poly(co-propoxylated bisphenol co-ethoxylated bisphenol co-maleate), poly(1,2-propylene maleate), poly(propoxylated bisphenol co-itaconate), poly(ethoxylated bisphenol co-itaconate), poly(butyloxylated bisphenol co-itaconate), poly(co-propoxylated bisphenol co-ethoxylated bisphenol co-itaconate), poly(1,2-propylene itaconate), and combinations thereof.

Furthermore, in embodiments, a crystalline polyester resin may be contained in the binding resin. The crystalline polyester resin may be synthesized from an acid (dicarboxylic acid) component and an alcohol (diol) component. In what follows, an "acid-derived component" indicates a constituent moiety that was originally an acid component before the synthesis of a polyester resin and an "alcohol-derived component" indicates a constituent moiety that was originally an alcoholic component before the synthesis of the polyester resin.

A "crystalline polyester resin" indicates one that shows not a stepwise endothermic amount variation but a clear endothermic peak in differential scanning calorimetry (DSC). However, a polymer obtained by copolymerizing the crystalline polyester main chain and at least one other component is also called a crystalline polyester if the amount of the other component is 50% by weight or less.

As the acid-derived component, an aliphatic dicarboxylic acid may be utilized, such as a straight chain carboxylic acid. Examples of straight chain carboxylic acids include oxalic acid, malonic acid, succinic acid, glutaric acid, adipic acid, pimelic acid, suberic acid, azelaic acid, sebacic acid, 1,9-nonanedicarboxylic acid, 1,10-decanedicarboxylic acid, 1,1-undecanedicarboxylic acid, 1,12-dodecanedicarboxylic acid, 1,13-tridecanedicarboxylic acid, 1,14-tetradecanedicarboxylic acid, 1,16-hexadecanedicarboxylic acid, and 1,18-octadecanedicarboxylic acid, as well as lower alkyl esters and acid anhydrides thereof. Among these, acids having 6 to 10 carbon atoms may be desirable for obtaining suitable crystal melting point and charging properties. In order to improve the crys-

tallinity, the straight chain carboxylic acid may be present in an amount of about 95% by mole or more of the acid component and, in embodiments, more than about 98% by mole of the acid component. Other acids are not particularly restricted, and examples thereof include conventionally known divalent carboxylic acids and dihydric alcohols, for example those described in "Polymer Data Handbook: Basic Edition" (Soc. Polymer Science, Japan Ed.: Baihukan). Specific examples of the monomer components include, as divalent carboxylic acids, dibasic acids such as phthalic acid, isophthalic acid, terephthalic acid, naphthalene-2,6-dicarboxylic acid, naphthalene-2,7-dicarboxylic acid, and cyclohexanedicarboxylic acid, and anhydrides and lower alkyl esters thereof, as well as combinations thereof, and the like. As the acid-derived component, a component such as a dicarboxylic acid-derived component having a sulfonic acid group may also be utilized. The dicarboxylic acid having a sulfonic acid group may be effective for obtaining excellent dispersion of a coloring agent such as a pigment. Furthermore, when a whole resin is emulsified or suspended in water to prepare a toner mother particle, a sulfonic acid group, may enable the resin to be emulsified or suspended without a surfactant. Examples of such dicarboxylic acids having a sulfonic group include, but are not limited to, sodium 2-sulfoterephthalate, sodium 5-sulfoisophthalate and sodium sulfosuccinate. Furthermore, lower alkyl esters and acid anhydrides of such dicarboxylic acids having a sulfonic group, for example, are also usable. Among these, sodium 5-sulfoisophthalate and the like may be desirable in view of the cost. The content of the dicarboxylic acid having a sulfonic acid group may be from about 0.1% by mole to about 2% by mole, in embodiments from about 0.2% by mole to about 1% by mole. When the content is more than about 2% by mole, the charging properties may be deteriorated. Here, "component mol %" or "component mole %" indicates the percentage when the total amount of each of the components (acid-derived component and alcohol-derived component) in the polyester resin is assumed to be 1 unit (mole).

As the alcohol component, aliphatic dialcohols may be used. Examples thereof include ethylene glycol, 1,3-propanediol, 1,4-butanediol, 1,5-pentanediol, 1,6-hexanediol, 1,7-heptanediol, 1,8-octanediol, 1,9-nonanediol, 1,10-decanediol, 1,11-dodecanediol, 1,12-undecanediol, 1,13-tridecanediol, 1,14-tetradecanediol, 1,18-octadecanediol and 1,20-eicosanediol. Among them, those having from about 6 to about 10 carbon atoms may be used to obtain desirable crystal melting points and charging properties. In order to raise crystallinity, it may be useful to use the straight chain dialcohols in an amount of about 95% by mole or more, in embodiments about 98% by mole or more.

Examples of other dihydric dialcohols which may be utilized include bisphenol A, hydrogenated bisphenol A, bisphenol A ethylene oxide adduct, bisphenol A propylene oxide adduct, 1,4-cyclohexanediol, 1,4-cyclohexanediethanol, diethylene glycol, propylene glycol, dipropylene glycol, 1,3-butanediol, neopentyl glycol, combinations thereof, and the like.

For adjusting the acid number and hydroxyl number, the following may be used: monoaliphatic acids such as acetic acid and benzoic acid; monohydric alcohols such as cyclohexanol and benzyl alcohol; benzenetricarboxylic acid, naphthalenetetracarboxylic acid, and anhydrides and lower alkylesters thereof; trivalent alcohols such as glycerin, trimethylolethane, trimethylolpropane, pentaerythritol, combinations thereof, and the like.

The crystalline polyester resins may be synthesized from a combination of components selected from the above-men-

tioned monomer components, by using conventional known methods. Exemplary methods include the ester exchange method and the direct polycondensation method, which may be used singularly or in a combination thereof. The molar ratio (acid component/alcohol component) when the acid component and alcohol component are reacted, may vary depending on the reaction conditions. The molar ratio is usually about 1/1 in direct polycondensation. In the ester exchange method, a monomer such as ethylene glycol, neopentyl glycol or cyclohexanediethanol, which may be distilled away under vacuum, may be used in excess.

#### Surfactants

Any suitable surfactants may be used for the preparation of the latex and wax dispersions according to the present disclosure. Depending on the emulsion system, any desired nonionic or ionic surfactant such as anionic or cationic surfactant may be contemplated.

Examples of suitable anionic surfactants include, but are not limited to, sodium dodecylsulfate, sodium dodecylbenzene sulfonate, sodium dodecylnaphthalenesulfate, dialkyl benzenealkyl sulfates and sulfonates, abitic acid, NEOGEN R® and NEOGEN SC® available from Kao, Tayca Power®, available from Tayca Corp., DOWFAX®, available from Dow Chemical Co., and the like, as well as mixtures thereof.

Anionic surfactants may be employed in any desired or effective amount, for example, at least about 0.01% by weight of total monomers used to prepare the latex polymer, at least about 0.1% by weight of total monomers used to prepare the latex polymer; and no more than about 10% by weight of total monomers used to prepare the latex polymer, although the amount can be outside of those ranges.

Examples of suitable cationic surfactants include, but are not limited to, dialkyl benzenealkyl ammonium chloride, lauryl trimethyl ammonium chloride, alkylbenzyl methyl ammonium chloride, alkyl benzyl dimethyl ammonium bromide, benzalkonium chloride, cetyl pyridinium bromide, C<sub>12</sub>, C<sub>15</sub> and C<sub>17</sub> trimethyl ammonium bromides, halide salts of quaternized polyoxyethylalkylamines, dodecylbenzyl triethyl ammonium chloride, MIRAPOL® and ALKAQUAT® (available from Alkaril Chemical Company), SANIZOL® (benzalkonium chloride, available from Kao Chemicals), and the like, as well as mixtures thereof.

Examples of suitable nonionic surfactants include, but are not limited to, polyvinyl alcohol, polyacrylic acid, methalose, methyl cellulose, ethyl cellulose, propyl cellulose, hydroxy ethyl cellulose, carboxy methyl cellulose, polyoxyethylene cetyl ether, polyoxyethylene lauryl ether, polyoxyethylene octyl ether, polyoxyethylene octylphenyl ether, polyoxyethylene oleyl ether, polyoxyethylene sorbitan monolaurate, polyoxyethylene stearyl ether, polyoxyethylene nonylphenyl ether, dialkylphenoxypoly(ethyleneoxy)ethanol (available from Rhone-Poulenc as IGEPAL CA-210®, IGEPAL CA-520®, IGEPAL CA-720®, IGEPAL CO-890®, IGEPAL CO-720®, IGEPAL CO-290®, IGEPAL CA-210®, ANTAROX 890®, and ANTAROX 897®) and the like, as well as mixtures thereof.

#### Initiators

Any suitable initiator or mixture of initiators may be selected in the latex process and the toner process. In embodiments, the initiator is selected from known free radical polymerization initiators. The free radical initiator can be any free radical polymerization initiator capable of initiating a free radical polymerization process and mixtures thereof, such free radical initiator being capable of providing free radical species on heating to above about 30° C.

Although water soluble free radical initiators are used in emulsion polymerization reactions, other free radical initiators also can be used. Examples of suitable free radical initiators include, but are not limited to, peroxides, such as, ammonium persulfate, hydrogen peroxide, acetyl peroxide, cumyl peroxide, tert-butyl peroxide, propionyl peroxide, benzoyl peroxide, chlorobenzoyl peroxide, dichlorobenzoyl peroxide, bromomethylbenzoyl peroxide, lauroyl peroxide, diisopropyl peroxycarbonate, tetralin hydroperoxide, 1-phenyl-2-methylpropyl-1-hydroperoxide and tert-butylhydroperoxide; pertriphenylacetate, tert-butyl performate; tert-butyl peracetate; tert-butyl perbenzoate; tert-butyl perphenylacetate; tert-butyl permethoxyacetate; tert-butyl per-N-(3-tolyl)carbamate; sodium persulfate; potassium persulfate, azo compounds, such as, 2,2'-azobisisopropane, 2,2'-dichloro-2,2'-azobisisopropane, 1,1'-azo(methylethyl)diacetate, 2,2'-azobis(2-amidinopropane)hydrochloride, 2,2'-azobis(2-amidinopropane)-nitrate, 2,2'-azobisisobutane, 2,2'-azobisisobutyramid, 2,2'-azobisisobutyronitrile, methyl 2,2'-azobis-2-methylpropionate, 2,2'-dichloro-2,2'-azobisisobutane, 2,2'-azobis-2-methylbutyronitrile, dimethyl 2,2'-azobisisobutyrate, 1,1'-azobis(sodium 1-methylbutyronitrile-3-sulfonate), 2-(4-methylphenylazo)-2-methylmalonodinitrile, 4,4'-azobis-4-cyanovaleic acid, 3,5-dihydroxymethylphenylazo-2-methylmalonodinitrile, 2-(4-bromophenylazo)-2-allylmalonodinitrile, 2,2'-azobis-2-methylvaleronitrile, dimethyl 4,4'-azobis-4-cyanovaleate, 2,2'-azobis-2,4-dimethylvaleronitrile, 1,1'-azobiscyclohexanenitrile, 2,2'-azobis-2-propylbutyronitrile, 1,1'-azobis-1-chlorophenylethane, 1,1'-azobis-1-cyclohexanecarbonitrile, 1,1'-azobis-1-cycloheptanenitrile, 1,1'-azobis-1-phenylethane, 1,1'-azobiscumene, ethyl 4-nitrophenylazobenzylcyanoacetate, phenylazodiphenylmethane, phenylazotriphenylmethane, 4-nitrophenylazotriphenylmethane, 1'-azobis-1,2-diphenylethane, poly(bisphenol A-4,4'-azobis-4-cyanopentano-ate) and poly(tetraethylene glycol-2,2'-azobisisobutyrate); 1,4-bis(pentaethylene)-2-tetrazene; 1,4-dimethoxycarbonyl-1,4-diphenyl-1-2-tetrazene and the like; and mixtures thereof.

More typical free radical initiators include, but are not limited to, ammonium persulfate, hydrogen peroxide, acetyl peroxide, cumyl peroxide, tert-butyl peroxide, propionyl peroxide, benzoyl peroxide, chlorobenzoyl peroxide, dichlorobenzoyl peroxide, bromomethylbenzoyl peroxide, lauroyl peroxide, sodium persulfate, potassium persulfate, diisopropyl peroxycarbonate and the like.

Based on total weight of the monomers to be polymerized, the initiator may be present in an amount from about 0.1% to about 5%, from about 0.4% to about 4%, from about 0.5% to about 3%, although may be present in greater or lesser amounts.

A chain transfer agent optionally may be used to control the polymerization degree of the latex, and thereby control the molecular weight and molecular weight distribution of the product latexes of the latex process and/or the toner process according to the present disclosure. As can be appreciated, a chain transfer agent can become part of the latex polymer.

#### Chain Transfer Agent

In embodiments, the chain transfer agent has a carbon-sulfur covalent bond. The carbon-sulfur covalent bond has an absorption peak in a wave number region ranging from 500 to 800  $\text{cm}^{-1}$  in an infrared absorption spectrum. When the chain transfer agent is incorporated into the latex and the toner made from the latex, the absorption peak may be changed, for example, to a wave number region of 400 to 4,000  $\text{cm}^{-1}$ .

Exemplary chain transfer agents include, but are not limited to, n-C<sub>3-15</sub> alkylmercaptans, such as, n-propylmercaptan,

n-butylmercaptan, n-amylmercaptan, n-hexylmercaptan, n-heptylmercaptan, n-octylmercaptan, n-nonylmercaptan, n-decylmercaptan and n-dodecylmercaptan; branched alkymercaptans, such as, isopropylmercaptan, isobutylmercaptan, s-butylmercaptan, tert-butylmercaptan, cyclohexylmercaptan, tert-hexadecylmercaptan, tert-laurylmercaptan, tert-nonylmercaptan, tert-octylmercaptan and tert-tetradecylmercaptan; aromatic ring-containing mercaptans, such as, allylmercaptan, 3-phenylpropylmercaptan, phenylmercaptan and mercaptotriphenylmethane; and so on. The terms, mercaptan and thiol may be used interchangeably to mean C—SH group.

Examples of such chain transfer agents also include, but are not limited to, dodecanethiol, butanethiol, isoctyl-3-mercaptopropionate, 2-methyl-5-t-butyl-thiophenol, carbon tetrachloride, carbon tetrabromide and the like.

Based on total weight of the monomers to be polymerized, the chain transfer agent may be present in an amount from about 0.1% to about 7%, from about 0.5% to about 6%, from about 1.0% to about 5%, although may be present in greater or lesser amounts.

In embodiments, a branching agent optionally may be included in the first/second monomer composition to control the branching structure of the target latex. Exemplary branching agents include, but are not limited to, decanediol diacrylate (ADOD), trimethylolpropane, pentaerythritol, trimellitic acid, pyromellitic acid and mixtures thereof.

Based on total weight of the monomers to be polymerized, the branching agent may be present in an amount from about 0% to about 2%, from about 0.05% to about 1.0%, from about 0.1% to about 0.8%, although may be present in greater or lesser amounts.

In the latex process and toner process of the disclosure, emulsification may be done by any suitable process, such as, mixing at elevated temperature. For example, the emulsion mixture may be mixed in a homogenizer set at about 200 to about 400 rpm and at a temperature of from about 40° C. to about 80° C. for a period of about 1 min to about 20 min.

Any type of reactor may be used without restriction. The reactor can include means for stirring the compositions therein, such as, an impeller. A reactor can include at least one impeller. For forming the latex and/or toner, the reactor can be operated throughout the process such that the impellers can operate at an effective mixing rate of about 10 to about 1,000 rpm.

Following completion of the monomer addition, the latex may be permitted to stabilize by maintaining the conditions for a period of time, for example for about 10 to about 300 min, before cooling. Optionally, the latex formed by the above process may be isolated by standard methods known in the art, for example, coagulation, dissolution and precipitation, filtering, washing, drying or the like.

The latex of the present disclosure may be selected for emulsion-aggregation-coalescence processes for forming toners, inks and developers by known methods. The latex of the present disclosure may be melt blended or otherwise mixed with various toner ingredients, such as, a wax dispersion, a coagulant, an optional silica, an optional charge enhancing additive or charge control additive, an optional surfactant, an optional emulsifier, an optional flow additive and the like. Optionally, the latex (e.g. around 40% solids) may be diluted to the desired solids loading (e.g. about 12 to about 15% by weight solids), before formulated in a toner composition.

Based on the total toner weight, the latex may be present in an amount from about 50% to about 100%, from about 60% to about 98%, from about 70% to about 95%, although may be

present in greater or lesser amounts. Methods of producing such latex resins may be carried out as described in the disclosure of U.S. Pat. No. 7,524,602, herein incorporated by reference in its entirety.

#### Colorants

Various known suitable colorants, such as dyes, pigments, mixtures of dyes, mixtures of pigments, mixtures of dyes and pigments and the like may be included in the toner. The colorant may be included in the toner in an amount of, for example, about 0.1 to about 35% by weight of the toner, from about 1 to about 15% percent of the toner, from about 3 to about 10% by weight of the toner, although amounts outside those ranges may be utilized.

As examples of suitable colorants, mention may be made of carbon black like REGAL 330®; magnetites, such as, Mobay magnetites MO8029™ and MO8060™; Columbian magnetites; MAPICO BLACKSTM, surface-treated magnetites; Pfizer magnetites CB4799™, CB5300™, CB5600™ and MCX6369™; Bayer magnetites, BAYFERROX 8600™ and 8610™; Northern Pigments magnetites, NP-604™ and NP-608™; Magnox magnetites TMB-100™ or TMB-104™; and the like. As colored pigments, there can be selected cyan, magenta, yellow, red, green, brown, blue or mixtures thereof. Generally, cyan, magenta or yellow pigments or dyes, or mixtures thereof, are used. The pigment or pigments can be water-based pigment dispersions.

Specific examples of pigments include SUNSPERSE 6000, FLEXIVERSE and AQUATONE water-based pigment dispersions from SUN Chemicals. HELIOGEN BLUE L6900™, D6840™, D7080™, D7020™, PYLAM OIL BLUE™, PYLAM OIL YELLOW™, PIGMENT BLUE 1™ available from Paul Uhlich & Company, Inc., PIGMENT VIOLET 1™, PIGMENT RED 48™, LEMON CHROME YELLOW DCC 1026™, E.D. TOLUIDINE RED™ and BON RED C™ available from Dominion Color Corporation, Ltd., Toronto, Ontario, NOVAPERM YELLOW FGL™, HOSTAPERM PINK E™ from Hoechst, CINQUASIA MAGENTA™ available from E.I. DuPont de Nemours & Company and the like. Colorants that can be selected are black, cyan, magenta, yellow and mixtures thereof. Examples of magentas are 2,9-dimethyl-substituted quinacridone and anthraquinone dye identified in the Color Index as CI-60710, CI Dispersed Red 15, diazo dye identified in the Color Index as CI-26050, CI Solvent Red 19 and the like. Illustrative examples of cyans include copper tetra(octadecyl sulfonamido) phthalocyanine, x-copper phthalocyanine pigment listed in the Color Index as CI-74160, CI Pigment Blue, Pigment Blue 15:3, Anthrathrene Blue, identified in the Color Index as CI-69810, Special Blue X-2137 and the like. Illustrative examples of yellows are diarylide yellow 3,3-dichlorobenzidine acetoacetanilides, a monoazo pigment identified in the Color Index as CI 12700, CI Solvent Yellow 16, a nitrophenyl amine sulfonamide identified in the Color Index as Foron Yellow SE/GLN, CI Dispersed Yellow 33 2,5-dimethoxy-4-sulfonanilide phenylazo-4'-chloro-2,5-dimethoxy acetoacetanilide and Permanent Yellow FGL. Colored magnetites, such as, mixtures of MAPICO BLACK™, and cyan components also may be selected as colorants. Other known colorants can be selected, such as, Levanyl Black A-SF (Miles, Bayer) and Sunperse Carbon Black LHD 9303 (Sun Chemicals), and colored dyes, such as, Neopen Blue (BASF), Sudan Blue OS (BASF), PV Fast Blue B2G01 (American Hoechst), Sunperse Blue BHD 6000 (Sun Chemicals), Irgalite Blue BCA (Ciba-Geigy), Paliogen Blue 6470 (BASF), Sudan III (Matheson, Coleman, Bell), Sudan II (Matheson, Coleman, Bell), Sudan IV (Matheson, Coleman, Bell), Sudan Orange G (Aldrich), Sudan Orange

220 (BASF), Paliogen Orange 3040 (BASF), Ortho Orange OR 2673 (Paul Uhlich), Paliogen Yellow 152, 1560 (BASF), Lithol Fast Yellow 0991K (BASF), Paliotol Yellow 1840 (BASF), Neopen Yellow (BASF), Novoperm Yellow FG 1 (Hoechst), Permanent Yellow YE 0305 (Paul Uhlich), Lumogen Yellow D0790 (BASF), Sunperse Yellow YHD 6001 (Sun Chemicals), Suco-Gelb L1250 (BASF), Suco-Yellow D1355 (BASF), Hostaperm Pink E (American Hoechst), Fanal Pink D4830 (BASF), Cinquasia Magenta (DuPont), 10 Lithol Scarlet D3700 (BASF), Toluidine Red (Aldrich), Scarlet for Thermoplast NSD PS PA (Ugine Kuhlmann of Canada), E.D. Toluidine Red (Aldrich), Lithol Rubine Toner (Paul Uhlich), Lithol Scarlet 4440 (BASF), Bon Red C (Dominion Color Company), Royal Brilliant Red RD-8192 (Paul Uhlich), Oracet Pink RF (Ciba-Geigy), Paliogen Red 3871K (BASF), Paliogen Red 3340 (BASF), Lithol Fast Scarlet L4300 (BASF), combinations of the foregoing and the like.

#### Wax

In addition to the polymer resin, the toners of the present disclosure also may contain a wax, which can be either a single type of wax or a mixture of two or more different waxes. A single wax can be added to toner formulations, for example, to improve particular toner properties, such as, toner particle shape, presence and amount of wax on the toner particle surface, charging and/or fusing characteristics, gloss, stripping, offset properties and the like. Alternatively, a combination of waxes can be added to provide multiple properties to the toner composition.

When included, the wax may be present in an amount of, 30 for example, from about 1 wt % to about 25 wt % of the toner particles, in embodiments, from about 5 wt % to about 20 wt % of the toner particles.

Waxes that may be selected include waxes having, for example, a weight average molecular weight of from about 35 500 to about 20,000, in embodiments from about 1,000 to about 10,000. Waxes that may be used include, for example, polyolefins, such as, polyethylene, polypropylene and polybutene waxes, such as, commercially available from Allied Chemical and Petrolite Corporation, for example POLY-40 WAX™ polyethylene waxes from Baker Petrolite, wax emulsions available from Michaelman, Inc. and the Daniels Products Company, EPOLENE N-15™ commercially available from Eastman Chemical Products, Inc., and VISCOL 550-P™, a low weight average molecular weight polypropylene 45 available from Sanyo Kasei K. K.; plant-based waxes, such as, carnauba wax, rice wax, candelilla wax, sumacs wax and jojoba oil; animal-based waxes, such as, beeswax; mineral-based waxes and petroleum-based waxes, such as, montan wax, ozokerite, ceresin, paraffin wax, microcrystalline wax 50 and Fischer-Tropsch wax; ester waxes obtained from higher fatty acid and higher alcohol, such as, stearyl stearate and behenyl behenate; ester waxes obtained from higher fatty acid and monovalent or multivalent lower alcohol, such as, butyl stearate, propyl oleate, glyceride monostearate, glyceride distearate, pentaerythritol tetra behenate; ester waxes obtained 55 from higher fatty acid and multivalent alcohol multimers, such as, diethyleneglycol monostearate, dipropylene glycol distearate, diglyceryl distearate and triglyceryl tetra stearate; sorbitan higher fatty acid ester waxes, such as, sorbitan monostearate, and cholesterol higher fatty acid ester waxes, such as, cholestryl stearate. Examples of functionalized 60 waxes that may be used include, for example, amines, amides, for example, AQUA SUPERSLIP 6550™ and SUPERSLIP 6530™ available from Micro Powder Inc., fluorinated waxes, for example, POLYFLUO 190™, POLYFLUO 200™, POLYSILK 19™ and POLYSILK 14™ available from Micro 65 Powder Inc., mixed fluorinated, amide waxes, for example,

MICROSPERSION 19<sup>TM</sup> available from Micro Powder Inc., imides, esters, quaternary amines, carboxylic acids or acrylic polymer emulsion, for example JONCRYL 74<sup>TM</sup> 89<sup>TM</sup>, 130<sup>TM</sup>, 537<sup>TM</sup> and 538<sup>TM</sup>, all available from SC Johnson Wax, and chlorinated polypropylenes and polyethylenes available from Allied Chemical and Petrolite Corporation and SC Johnson wax. Mixtures and combinations of the foregoing waxes also may be used in embodiments. Waxes may be included as, for example, fuser roll release agents.

#### Toner Preparation

The toner particles may be prepared by any method within the purview of one skilled in the art. Although embodiments relating to toner particle production are described below with respect to emulsion-aggregation processes, any suitable method of preparing toner particles may be used, including chemical processes, such as suspension and encapsulation processes disclosed in U.S. Pat. No. 5,290,654 and U.S. Pat. No. 5,302,486, the disclosure of each which is hereby incorporated by reference in their entirety. In embodiments, toner compositions and toner particles may be prepared by aggregation and coalescence processes in which smaller-sized resin particles are aggregated to the appropriate toner particle size and then coalesced to achieve the final toner particle shape and morphology.

In embodiments, toner compositions may be prepared by emulsion-aggregation processes, such as, a process that includes aggregating a mixture of an optional wax and any other desired or required additives, and emulsions including the resins described above, optionally with surfactants, as described above, and then coalescing the aggregate mixture. A mixture may be prepared by adding an optional wax or other materials, which optionally also may be in a dispersion (s) including a surfactant, to the emulsion, which may be a mixture of two or more emulsions containing the resin. The pH of the resulting mixture may be adjusted by an acid (i.e., a pH adjustor) such as, for example, acetic acid, nitric acid or the like. In embodiments, the pH of the mixture may be adjusted to from about 2 to about 4.5. Additionally, in embodiments, the mixture may be homogenized. If the mixture is homogenized, homogenization may be accomplished by mixing at about 600 to about 4,000 revolutions per minute (rpm). Homogenization may be accomplished by any suitable means, including, for example, with an IKA ULTRA TUR-RAX T50 probe homogenizer.

Following preparation of the above mixture, an aggregating agent may be added to the mixture. Suitable aggregating agents include, for example, aqueous solutions of a divalent cation or a multivalent cation material. The aggregating agent may be, for example, polyaluminum halides, such as, poly-aluminum chloride (PAC), or the corresponding bromide, fluoride or iodide, polyaluminum silicates, such as, polyaluminum sulfosilicate (PASS), and water soluble metal salts including aluminum chloride, aluminum nitrite, aluminum sulfate, potassium aluminum sulfate, calcium acetate, calcium chloride, calcium nitrite, calcium oxybate, calcium sulfate, magnesium acetate, magnesium nitrate, magnesium sulfate, zinc acetate, zinc nitrate, zinc sulfate, zinc chloride, zinc bromide, magnesium bromide, copper chloride, copper sulfate, and combinations thereof. In embodiments, the aggregating agent may be added to the mixture at a temperature that is below the glass transition temperature ( $T_g$ ) of the resin.

The aggregating agent may be added to the mixture to form a toner in an amount of, for example, from about 0.1 parts per hundred (pph) to about 1 pph, in embodiments, from about 0.25 pph to about 0.75 pph.

The gloss of a toner may be influenced by the amount of retained metal ion, such as, Al<sup>3+</sup>, in the particle. The amount

of retained metal ion may be adjusted further by the addition of ethylene diamine tetraacetic acid (EDTA). In embodiments, the amount of retained metal ion, for example, Al<sup>3+</sup>, in toner particles of the present disclosure may be from about 0.1 pph to about 1 pph, in embodiments, from about 0.25 pph to about 0.8 pph.

The disclosure also provides a melt mixing process to produce low cost and safe cross-linked thermoplastic binder resins for toner compositions which have, for example, low

10 fix temperature and/or high offset temperature, and which may show minimized or substantially no vinyl offset. In the process, unsaturated base polyester resins or polymers are melt blended, that is, in the molten state under high shear conditions producing substantially uniformly dispersed toner 15 constituents, and which process provides a resin blend and toner product with optimized gloss properties (see, e.g., U.S. Pat. No. 5,556,732, herein incorporated by reference in its entirety). By, "highly cross-linked," is meant that the polymer involved is substantially cross-linked, that is, equal to or 20 above the gel point. As used herein, "gel point," means the point where the polymer is no longer soluble in solution (see, e.g., U.S. Pat. No. 4,457,998, herein incorporated by reference in its entirety).

To control aggregation and coalescence of the particles, in 25 embodiments, the aggregating agent may be metered into the mixture over time. For example, the agent may be metered into the mixture over a period of from about 5 to about 240 min, in embodiments, from about 30 to about 200 min. Addition of the agent may also be done while the mixture is 30 maintained under stirred conditions, in embodiments from about 50 rpm to about 1,000 rpm, in embodiments, from about 100 rpm to about 500 rpm, and at a temperature that is below the  $T_g$  of the resin.

The particles may be permitted to aggregate until a predetermined desired particle size is obtained. A predetermined desired size refers to the desired particle size as determined prior to formation, with particle size monitored during the growth process as known in the art until such particle size is achieved. Samples may be taken during the growth process 35 and analyzed, for example with a Coulter Counter, for average particle size. The aggregation thus may proceed by maintaining the elevated temperature, or slowly raising the temperature to, for example, from about 40° C. to about 100° C., and holding the mixture at that temperature for a time from 40 about 0.5 hr to about 6 hr, in embodiments, from about 1 hr to about 5 hr, while maintaining stirring, to provide the aggregated particles. Once the predetermined desired particle size is obtained, the growth process is halted. In embodiments, the predetermined desired particle size is within the toner particle 45 size ranges mentioned above. In embodiments, the particle size may be about 5.0 to about 6.0  $\mu$ m, about 6.0 to about 6.5  $\mu$ m, about 6.5 to about 7.0  $\mu$ m, about 7.0 to about 7.5  $\mu$ m.

Growth and shaping of the particles following addition of the aggregating agent may be accomplished under any suitable conditions. For example, the growth and shaping may be conducted under conditions in which aggregation occurs separate from coalescence. For separate aggregation and coalescence stages, the aggregation process may be conducted under shearing conditions at an elevated temperature, for 55 example from about 40° C. to about 90° C., in embodiments, from about 45° C. to about 80° C., which may be below the  $T_g$  of the resin.

Toners may possess favorable charging characteristics when exposed to extreme RH conditions. The low humidity 60 zone (C zone) may be about 12° C./15% RH, while the high humidity zone (A zone) may be about 28° C./85% RH. Toners of the disclosure may possess a parent toner charge per mass

ratio (Q/M) of from about  $-5 \mu\text{C/g}$  to about  $-80 \mu\text{C/g}$ , in embodiments, from about  $-10 \mu\text{C/g}$  to about  $-70 \mu\text{C/g}$ , and a final toner charging after surface additive blending of from  $-15 \mu\text{C/g}$  to about  $-60 \mu\text{C/g}$ , in embodiments, from about  $-20 \mu\text{C/g}$  to about  $-55 \mu\text{C/g}$ .

#### Shell Resin

In embodiments, a shell may be applied to the formed aggregated toner particles. Any resin described above as suitable for the core resin may be utilized as the shell resin. The shell resin may be applied to the aggregated particles by any method within the purview of those skilled in the art. In embodiments, the shell resin may be in an emulsion including any surfactant described herein. The aggregated particles described above may be combined with said emulsion so that the resin forms a shell over the formed aggregates. In embodiments, an amorphous polyester may be utilized to form a shell over the aggregates to form toner particles having a core-shell configuration.

Toner particles can have a size of diameter of from about 4 to about  $8 \mu\text{m}$ , in embodiments, from about 5 to about  $7 \mu\text{m}$ , the optimal shell component may be about 26 to about 30% by weight of the toner particles.

Alternatively, a thicker shell may be desirable to provide desirable charging characteristics due to the higher surface area of the toner particle. Thus, the shell resin may be present in an amount from about 30% to about 40% by weight of the toner particles, in embodiments, from about 32% to about 38% by weight of the toner particles, in embodiments, from about 34% to about 36% by weight of the toner particles.

In embodiments, a photoinitiator may be included in the shell. Thus, the photoinitiator may be in the core, the shell, or both. The photoinitiator may be present in an amount of from about 1% to about 5% by weight of the toner particles, in embodiments, from about 2% to about 4% by weight of the toner particles.

Emulsions may have a solids loading of from about 5% solids by weight to about 20% solids by weight, in embodiments, from about 12% solids by weight to about 17% solids by weight.

Once the desired final size of the toner particles is achieved, the pH of the mixture may be adjusted with a base (i.e., a pH adjustor) to a value of from about 6 to about 10, and in embodiments from about 6.2 to about 7. The adjustment of the pH may be utilized to freeze, that is to stop, toner growth. The base utilized to stop toner growth may include any suitable base, such as, for example, alkali metal hydroxides, such as, for example, sodium hydroxide, potassium hydroxide, ammonium hydroxide, combinations thereof and the like. In embodiments, EDTA may be added to help adjust the pH to the desired values noted above. The base may be added in amounts from about 2 to about 25% by weight of the mixture, in embodiments, from about 4 to about 10% by weight of the mixture. In embodiments, the shell has a higher  $T_g$  than the aggregated toner particles.

#### Coalescence

Following aggregation to the desired particle size, with the optional formation of a shell as described above, the particles then may be coalesced to the desired final shape, the coalescence being achieved by, for example, heating the mixture to a temperature of from about  $55^\circ \text{C}$ . to about  $100^\circ \text{C}$ ., in embodiments from about  $65^\circ \text{C}$ . to about  $75^\circ \text{C}$ ., which may be below the melting point of a crystalline resin to prevent plasticization. Higher or lower temperatures may be used, it being understood that the temperature is a function of the resins used.

Coalescence may proceed over a period of from about 0.1 to about 9 hr, in embodiments, from about 0.5 to about 4 hr.

After coalescence, the mixture may be cooled to room temperature, such as from about  $20^\circ \text{C}$ . to about  $25^\circ \text{C}$ . The cooling may be rapid or slow, as desired. A suitable cooling method may include introducing cold water to a jacket around the reactor. After cooling, the toner particles optionally may be washed with water and then dried. Drying may be accomplished by any suitable method, for example, freeze drying.

#### Carriers

Various suitable solid core or particle materials can be utilized for the carriers and developers of the present disclosure. Characteristic particle properties include those that, in embodiments, will enable the toner particles to acquire a positive charge or a negative charge, and carrier cores that provide desirable flow properties in the developer reservoir present in an electrophotographic imaging apparatus. Other desirable properties of the core include, for example, suitable magnetic characteristics that permit magnetic brush formation in magnetic brush development processes; desirable mechanical aging characteristics; and desirable surface morphology to permit high electrical conductivity of any developer including the carrier and a suitable toner.

Examples of carrier particles or cores that can be utilized include iron and/or steel, such as, atomized iron or steel powders available from Hoeganaes Corporation or Pomaton S.p.A (Italy); ferrites, such as, Cu/Zn-ferrite containing, for example, about 11% copper oxide, about 19% zinc oxide, and about 70% iron oxide, including those commercially available from D.M. Steward Corporation or Powdertech Corporation, Ni/Zn-ferrite available from Powdertech Corporation, Sr (strontium)-ferrite, containing, for example, about 14% strontium oxide and about 86% iron oxide, commercially available from Powdertech Corporation, and Ba-ferrite; magnetites, including those commercially available from, for example, Hoeganaes Corporation (Sweden); nickel; combinations thereof, and the like. In embodiments, the polymer particles obtained can be used to coat carrier cores of any known type by various known methods, and which carriers then are incorporated with a known toner to form a developer for electrophotographic printing. Other suitable carrier cores are illustrated in, for example, U.S. Pat. Nos. 4,937,166, 4,935,326 and U.S. Pat. No. 7,014,971, the disclosure of each which is hereby incorporated by reference in their entirety, and may include granular zircon, granular silicon, glass, silicon dioxide, combinations thereof, and the like. In embodiments, suitable carrier cores may have an average particle size of, for example, from about  $20 \mu\text{m}$  to about  $400 \mu\text{m}$  in diameter, in embodiments, from about  $40 \mu\text{m}$  to about  $200 \mu\text{m}$  in diameter.

In embodiments, a ferrite may be utilized as the core, including a metal, such as, iron and at least one additional metal, such as, copper, zinc, nickel, manganese, magnesium, calcium, lithium, strontium, zirconium, titanium, tantalum, bismuth, sodium, potassium, rubidium, cesium, strontium, barium, yttrium, lanthanum, hafnium, vanadium, niobium, aluminum, gallium, silicon, germanium, antimony, combinations thereof and the like.

In some embodiments, the carrier coating may include a conductive component. Suitable conductive components include, for example, carbon black.

There may be added to the carrier a number of additives, for example, charge enhancing additives, including particulate amine resins, such as, melamine, and certain fluoropolymer powders, such as alkyl-amino acrylates and methacrylates, polyamides, and fluorinated polymers, such as polyvinylidene fluoride and poly(tetrafluoroethylene) and fluoroalkyl methacrylates, such as 2,2,2-trifluoroethyl methacrylate. Other charge enhancing additives which may be utilized include

quaternary ammonium salts, including distearyl dimethyl ammonium methyl sulfate (DDAMS), bis[1-[(3,5-disubstituted-2-hydroxyphenyl)azo]-3-(mono-substituted)-2-naphthalenolato(2-)]chromate(1-), ammonium sodium and hydrogen (TRH), cetyl pyridinium chloride (CPC), FANAL PINK® D4830, combinations thereof, and the like, and other effective known charge agents or additives. The charge additive components may be selected in various effective amounts, such as from about 0.5 wt % to about 20 wt %, from about 1 wt % to about 3 wt %, based, for example, on the sum of the weights of polymer/copolymer, conductive component, and other charge additive components. The addition of conductive components can act to further increase the negative triboelectric charge imparted to the carrier, and therefore, further increase the negative triboelectric charge imparted to the toner in, for example, an electrophotographic development subsystem. The components may be included by roll mixing, tumbling, milling, shaking, electrostatic powder cloud spraying, fluidized bed, electrostatic disc processing, and an electrostatic curtain, as described, for example, in U.S. Pat. No. 6,042,981, the disclosure of which hereby is incorporated by reference in its entirety, and wherein the carrier coating is fused to the carrier core in either a rotary kiln or by passing through a heated extruder apparatus.

Conductivity can be important for semiconductive magnetic brush development to enable good development of solid areas which otherwise may be weakly developed. Addition of a polymeric coating of the present disclosure, optionally with a conductive component such as carbon black, can result in carriers with decreased developer triboelectric response with change in relative humidity of from about 20% to about 90%, in embodiments, from about 40% to about 80%, that the charge is more consistent when the relative humidity is changed. Thus, there is less decrease in charge at high relative humidity reducing background toner on the prints, and less increase in charge and subsequently less loss of development at low relative humidity, resulting in such improved image quality performance due to improved optical density.

As noted above, in embodiments the polymeric coating may be dried, after which time it may be applied to the core carrier as a dry powder. Powder coating processes differ from conventional solution coating processes. Solution coating requires a coating polymer whose composition and molecular weight properties enable the resin to be soluble in a solvent in the coating process. That requires relatively low  $M_w$  components as compared to powder coating. The powder coating process does not require solvent solubility, but does require the resin coated as a particulate with a particle size of from about 10 nm to about 2  $\mu\text{m}$ , in embodiments, from about 30 nm to about 1  $\mu\text{m}$ , in embodiments, from about 50 nm to about 500 nm.

Examples of processes which may be utilized to apply the powder coating include, for example, combining the carrier core material and resin coating by cascade roll mixing, tumbling, milling, shaking, electrostatic powder cloud spraying, fluidized bed, electrostatic disc processing, electrostatic curtains, combinations thereof and the like. When resin coated carrier particles are prepared by a powder coating process, the majority of the coating materials may be fused to the carrier surface, thereby reducing the number of toner impaction sites on the carrier. Fusing of the polymeric coating may occur by mechanical impaction, electrostatic attraction, combinations thereof and the like.

Following application of the resin to the core, heating may be initiated to permit flow of the coating material over the surface of the carrier core. The concentration of the coating material, in embodiments, powder particles, and the param-

eters of the heating may be selected to enable the formation of a continuous film of the coating polymers on the surface of the carrier core, or permit only selected areas of the carrier core to be coated. In embodiments, the carrier with the polymeric powder coating may be heated to a temperature of from about 170° C. to about 280° C., in embodiments from about 190° C. to about 240° C., for a period of time of, for example, from about 10 min to about 180 min, in embodiments, from about 15 min to about 60 min, to enable the polymer coating to melt and to fuse to the carrier core particles. Following incorporation of the powder on the surface of the carrier, heating may be initiated to permit flow of the coating material over the surface of the carrier core. In embodiments, the powder may be fused to the carrier core in either a rotary kiln or by passing through a heated extruder apparatus, see, for example, U.S. Pat. No. 6,355,391, the disclosure of which hereby is incorporated by reference in its entirety.

In embodiments, the coating coverage encompasses from about 10% to about 100% of the carrier core. When selected areas of the metal carrier core remain uncoated or exposed, the carrier particles may possess electrically conductive properties when the core material is a metal.

The coated carrier particles may then be cooled, in embodiments to room temperature, and recovered for use in forming developer.

In embodiments, carriers of the present disclosure may include a core, in embodiments, a ferrite core, having a size of from about 20  $\mu\text{m}$  to about 100  $\mu\text{m}$ , in embodiments, from about 30  $\mu\text{m}$  to about 75  $\mu\text{m}$ , coated with from about 0.5% to about 10% by weight, in embodiments, from about 0.7% to about 5% by weight, of the polymer coating of the present disclosure, optionally including carbon black.

Thus, with the carrier compositions and processes of the present disclosure, there can be formulated developers with selected high triboelectric charging characteristics and/or conductivity values utilizing a number of different combinations.

#### Developers

The toner particles thus formed may be formulated into a developer composition. The toner particles may be mixed with carrier particles to achieve a two component developer composition. The toner concentration in the developer may be from about 1% to about 25% by weight of the total weight of the developer, in embodiments, from about 2% to about 15% by weight of the total weight of the developer.

#### Imaging

The toners can be utilized for electrophotographic processes, including those disclosed in U.S. Pat. No. 4,295,990, the disclosure of which is hereby incorporated by reference in its entirety. In embodiments, any known type of image development system may be used in an image developing device, including, for example, magnetic brush development, hybrid scavengerless development (HSD) and the like. Those and similar development systems are within the purview of those skilled in the art.

It is envisioned that the toners of the present disclosure may be used in any suitable procedure for forming an image with a toner, including in applications other than xerographic applications.

Utilizing the toners of the present disclosure, images may be formed on substrates, including flexible substrates, having a toner pile height of from about 1  $\mu\text{m}$  to about 6  $\mu\text{m}$ , in embodiments, from about 2  $\mu\text{m}$  to about 4.5  $\mu\text{m}$ , in embodiments, from about 2.5 to about 4.2  $\mu\text{m}$ .

In embodiments, the toner of the present disclosure may be used for a xerographic print protective composition that provides overprint coating properties including, but not limited

to, thermal and light stability and smear resistance, particularly in commercial print applications. More specifically, such overprint coating as envisioned has the ability to permit overwriting, reduce or prevent thermal cracking, improve fusing, reduce or prevent document offset, improve print performance and protect an image from sun, heat and the like. In embodiments, the overprint compositions may be used to improve the overall appearance of xerographic prints due to the ability of the compositions to fill in the roughness of xerographic substrates and toners, thereby forming a level film and enhancing glossiness.

The following Examples are submitted to illustrate embodiments of the disclosure. The Examples are intended to be illustrative only and are not intended to limit the scope of the disclosure. Also, parts and percentages are by weight unless otherwise indicated. As used herein, "room temperature," refers to a temperature of from about 20° C. to about 30° C.

## EXAMPLES

The examples set forth herein below are being submitted to illustrate embodiments of the present disclosure. These examples are intended to be illustrative only and are not intended to limit the scope of the present disclosure. Also, parts and percentages are by weight (wt %) unless otherwise indicated. Comparative examples and data are also provided.

### Example 1

#### Synthesis and Characterization of Alumina Nanotubes

Synthesis of alumina nanotubes have been reported by Lihong Qu, Changqing He, Yue Yang, Yanli He, Zhongmin Liu, "Hydrothermal synthesis of alumina nanotubes templated by anionic surfactant", Materials Letters, Volume 59, Issues 29-30, December 2005, Pages 4034-4037, which is hereby incorporated by reference in its entirety.

As a prophetic example alumina nanotubes of 6 nm to 8 nm in outer diameter and up to 200 nm in length can be prepared. To form alumina nanotubes, 2.8 g of sodium dodecyl sulfonate can be dissolved into 70 g of distilled water at 50° C. to prepare solution A. Then 22.9 g of  $\text{Al}(\text{NO}_3)_3 \cdot 9\text{H}_2\text{O}$  can be dissolved in 40 g of distilled water at room temperature to achieve solution B. Solution B can then be slowly added into solution A under stirring, and the mixture can be continuously stirred for several minutes at 50° C. Thereafter, 12.0 g of aqueous ammonia can be dripped into the mixture until pH value of 5.0-5.5. After being stirred for additional several minutes, the resulting suspension can be transferred into a Teflon-lined autoclave (100 ml), and can be heated at 120° C. for 90 h. After the completion of hydrothermal treatment, the autoclave can be cooled down to room temperature naturally, and the solid product can be recovered by centrifuge, washed several times with a solution consisting of distilled water and 95% ethanol, and finally dried at 50° C. overnight. The template in the solids can be removed by calcinations and extraction, respectively. During calcinations, the sample can be heated in air from room temperature to a certain temperature in the range of 500-800° C. with a temperature ramp of 1° C.  $\text{min}^{-1}$ , and kept at that temperature for 5 h. 0.2 M ethanol solution of ammonium acetate can be used to perform the solvent extraction at room temperature for 4 days while stirring.

The length, outer and inner diameter of the silica nanotubes can be characterized via high-magnification TEM analysis

performed with a JEOL-JEM-2000EX apparatus with an accelerating voltage of 100.0 kV.

### Example 2

#### Toner and Developer Preparation

A prophetic example of an additive package utilizing AlNT is shown in Table 1 below.

TABLE 1

| Component         | Wt %   |
|-------------------|--------|
| Parent Particle   | 94.28% |
| RX50              | 0.86%  |
| RY50              | 1.29%  |
| STT100H           | 0.88%  |
| Alumina Nanotubes | 1.73%  |
| ZnSt Fine Powder  | 0.18%  |
| PMMA              | 0.50%  |
| CeO2              | 0.28%  |

Toners can be blended in a 10 liter Henschel mixer for about 5 minutes at about 2640 rpm. Developers can be prepared with Xerox 700 carrier at 8% toner concentration. Toners and carriers can be weighed out to a total of about 450 grams of developer in a 1 liter glass jar. The glass jar can be sealed and mixed for 10 minutes on a Turbula mixer. These toners and developers then can be used in a Xerox 700 machine for printing.

#### Characterization of Developer Charge

Developers can be prepared by adding 0.5 grams toner to 10 grams of Xerox 700 carrier. A duplicate developer sample pair can be prepared for each toner evaluated. One developer of the pair can be conditioned overnight in A-zone (28° C./85% RH), and the other can be conditioned overnight in the C-zone (10° C./15% RH). The next day, the developer samples can be sealed and agitated for about 2 minutes and then for about 1 hour using a Turbula mixer. After mixing, the triboelectric charge of the toner can be measured using a charge spectrograph with a 100 V/cm field. The toner charge (q/d) can be measured visually as the midpoint of the toner charge distribution. The charge can be reported in millimeters of displacement from the zero line (mm displacement can be converted to femtocoulombs/micron (FC/ $\mu\text{m}$ ) by multiplying by 0.092).

Following about 1 hour of mixing, an additional 0.5 grams of toner can be added to the already charged developer, and mixed for an additional 15 seconds, where a q/d displacement can be measured again, and then mixed for an additional 45 seconds (total 1 minute of mixing), and again a q/d displacement can be measured. This procedure will measure the toner admix.

The Q/M can also be measured by the total blow-off method, a method primarily used for the measurement of dual component toner, which is in the purview of those skilled in the art. In the blow-off method, the particles are first deposited, and then blown off using an air stream to characterize triboelectric properties of particles relative to different surfaces.

Alumina nanotubes prepared in accordance with an embodiment of the present teachings may have the following characteristics desirable for their use as a toner additive. In embodiments, the alumina nanotubes provide excellent toner flow and blocking, the latter the toner flow at high temperature. In embodiments, the alumina nanotubes provide reduced impaction of the other additives in the toner compo-

sition, enabling those other additives to remain effective in providing excellent toner charge and excellent relative humidity resistance, such that the excellent charge is maintained at high relative humidity. In addition, the alumina nanotubes, in embodiments, provide excellent adhesion of the additive to the toner particle, preventing loss of the additive which can lead to contamination of other subsystems, where such loss of additive leads to streaks, spots or areas of low density, or background in the prints. The additive attachment may be measured by the AAFD, where a higher value of AAFD indicates better additive attachment to the toner surface. In embodiments, the alumina nanotubes provide negative or positive charging to the toner, and thus can be used with other toner additives and charge enhancing additives, to control the charge level of the toner in the electrophotographic printer, thus enabling excellent dark solid images without background on the print, with excellent print quality, such as low image noise in the print over different environmental conditions.

Notwithstanding that the numerical ranges and parameters setting forth the broad scope of the present teachings are approximations, the numerical values set forth in the specific examples are reported as precisely as possible. Any numerical value, however, inherently contains certain errors necessarily resulting from the standard deviation found in their respective testing measurements. Moreover, all ranges disclosed herein are to be understood to encompass any and all sub-ranges subsumed therein. For example, a range of "less than 10" can include any and all sub-ranges between (and including) the minimum value of zero and the maximum value of 10, that is, any and all sub-ranges having a minimum value of equal to or greater than zero and a maximum value of equal to or less than 10, e.g., 1 to 5. In certain cases, the numerical values as stated for the parameter can take on negative values. In this case, the example value of range stated as "less than 10" can assume negative values, e.g. -1, -2, -3, -10, -20, -30, etc.

While the present teachings have been illustrated with respect to one or more implementations, alterations and/or modifications can be made to the illustrated examples without departing from the spirit and scope of the appended claims. For example, it will be appreciated that while the process is described as a series of acts or events, the present teachings are not limited by the ordering of such acts or events. Some acts may occur in different orders and/or concurrently with other acts or events apart from those described herein. Also, not all process stages may be required to implement a methodology in accordance with one or more aspects or embodiments of the present teachings. It will be appreciated that structural components and/or processing stages can be added or existing structural components and/or processing stages can be removed or modified. Further, one or more of the acts depicted herein may be carried out in one or more separate acts and/or phases. Furthermore, to the extent that the terms "including," "includes," "having," "has," "with," or variants thereof are used in either the detailed description and the claims, such terms are intended to be inclusive in a manner similar to the term "comprising." The term "at least one of" is used to mean one or more of the listed items can be selected. Further, in the discussion and claims herein, the term "on" used with respect to two materials, one "on" the other, means at least some contact between the materials, while "over" means the materials are in proximity, but possibly with one or more additional intervening materials such that contact is possible but not required. Neither "on" nor "over" implies any directionality as used herein. The term "conformal" describes a coating material in which angles of the underlying material are preserved by the conformal material. The term "about"

indicates that the value listed may be somewhat altered, as long as the alteration does not result in nonconformance of the process or structure to the illustrated embodiment. Finally, "exemplary" indicates the description is used as an example, rather than implying that it is an ideal. Other embodiments of the present teachings will be apparent to those skilled in the art from consideration of the specification and practice of the disclosure herein. It is intended that the specification and examples be considered as exemplary only, with a true scope and spirit of the present teachings being indicated by the following claims.

Terms of relative position as used in this application are defined based on a plane parallel to the conventional plane or working surface of a workpiece, regardless of the orientation of the workpiece. The term "horizontal" or "lateral" as used in this application is defined as a plane parallel to the conventional plane or working surface of a workpiece, regardless of the orientation of the workpiece. The term "vertical" refers to a direction perpendicular to the horizontal. Terms such as "on," "side" (as in "sidewall"), "higher," "lower," "over," "top," and "under" are defined with respect to the conventional plane or working surface being on the top surface of the workpiece, regardless of the orientation of the workpiece.

25 The invention claimed is:

1. A toner composition, comprising:  
toner particles comprising a resin and a colorant; and  
one or more surface additives applied to a surface of the  
toner particles, the one or more surface additives comprising alumina nanotubes.

20 2. The toner composition of claim 1, wherein the one or more surface additives further comprise at least one of a particulate silica, a particulate titania, and mixtures thereof.

3. The toner composition of claim 2, wherein the one or  
35 more surface additives comprise a particulate titania and the particulate titania has an anatase or rutile structure.

4. The toner composition of claim 3, wherein:  
the toner composition comprises at least one of a silica and  
a titania, wherein each of the at least one of the silica and  
the titania comprises between about 0.1 wt % and 4 wt %  
of a total weight of the toner composition; and  
the alumina nanotubes comprise between 0.1 wt % and 4  
wt % of the total weight of the toner composition.

5. The toner composition of claim 2, wherein the at least  
45 one of the particulate silica, the particulate titania, and the mixtures thereof are present in an amount ranging from about 0.1 to about 5 percent by weight of a total weight of the toner composition.

6. The toner composition of claim 1, wherein the alumina  
50 nanotubes comprise between 0.1 wt % to about 5.0 wt % of  
the toner composition.

7. The toner composition of claim 1, wherein the toner  
composition further comprises at least one material selected  
55 from the group consisting of silica nanotubes, titania nanotubes, and combinations thereof.

8. The toner composition of claim 7, wherein:  
the alumina nanotubes comprises between 0.1 wt % and 5  
wt % of the toner composition; and  
the at least one material selected from the group consisting  
of silica nanotubes, titania nanotubes, and combinations  
thereof comprises between 0.1 wt % and 4 wt % of the  
toner composition.

9. The toner composition of claim 7, wherein:  
the toner composition comprises both silica nanotubes and  
titania nanotubes;  
the silica nanotubes comprise between 0.1 wt % and 4 wt %  
of the toner composition;

## 29

the titania nanotubes comprise between 0.1 wt % and 4 wt % of the toner composition; and the alumina nanotubes comprise between 0.1 wt % and 4 wt % of the toner composition.

10. The toner composition of claim 1, further comprising one or more photoreceptor cleaning additives, where the one or more surface additives further comprise a particulate cerium dioxide, a fluoropolymer, a particulate comprised of a fluoropolymer, a particulate comprised of polytetrafluoroethylene, a particulate comprised of a polymethylmethacrylate, a particulate comprised of a metal stearate, a particulate comprised of zinc stearate, aluminum stearate or calcium stearate and mixtures thereof.

11. The toner composition of claim 1, wherein the alumina nanotubes have an average particle diameter of from about from about 5 nm to about 100 nm.

12. The toner composition of claim 11, wherein the alumina nanotubes have an average particle diameter of from about from about 5 nm to about 50 nm.

13. The toner composition of claim 1, wherein the alumina nanotubes have an average particle length of from about from about 50 nm to about 2 microns.

14. The toner composition of claim 13, wherein the alumina nanotubes have an average particle length of from about from about 100 nm to about 1 micron.

15. The toner composition of claim 1 having a percent toner cohesion from about 10% to about 78%.

16. The toner composition of claim 1, wherein the toner composition comprises an Additive Adhesion Force Distribu-

## 30

tion (AAFD) percent value of greater than 40 percent after from about 2.5 to about 3 minutes of sonification and 3 kilojoules of energy.

17. A toner composition, comprising:  
5 toner particles comprising a resin and a colorant; and one or more surface additives applied to a surface of the toner particles, the one or more surface additives comprising alumina nanotubes, wherein the toner composition has a high charge of from about -15 microcoulomb per gram to about -80 microcoulomb per gram and a low relative humidity sensitivity ratio of from about 1 to about 2.

18. The toner composition of claim 17, wherein the alumina nanotubes have an average particle diameter of from about from about 5 nm to about 100 nm and an average particle length of from about from about 50 nm to about 2 microns.

19. A developer comprising:  
a toner composition; and  
20 a toner carrier, wherein the toner composition comprises toner particles comprising a resin and a colorant, and one or more surface additives applied to a surface of the toner particles, the one or more surface additives comprising alumina nanotubes.

25 20. The developer of claim 19, wherein the toner composition is an emulsion aggregation toner composition.

21. The developer of claim 19, wherein the toner composition is prepared by physical methods.

\* \* \* \* \*